# EUROPEAN PATENT SPECIFICATION

(11) **EP 0 439 337 B1**
(45) Date of publication and mention of the grant of the patent: **05.04.1995**
(21) Application number: 91300505.4
(22) Date of filing: 23.01.1991
(51) Int. Cl.: H01Q 17/00

(54) **Broad-band wave absorber**
Breitbandiger Wellenabsorber
Absorbeur d'ondes à large bande

(30) Priority: 25.01.1990 JP 15798/90; 02.02.1990 JP 23818/90; 08.06.1990 JP 150690/90; 20.06.1990 JP 162403/90
(43) Date of publication of application: 31.07.1991
(73) Proprietor: Naito, Yoshiyuki, Yamato-Shi Kanagawa-Ken (JP); Takahashi, Michiharu, Yachiyo-Shi Chiba-Ken (JP)
(72) Inventor: Naito, Yoshiyuki, Yamato-Shi Kanagawa-Ken (JP); Takahashi, Michiharu, Yachiyo-Shi Chiba-Ken (JP)
(74) Representative: Palmer, Roger

(56) References cited:
- GB-A- 776 158
- GB-A- 1 170 420
- US-A- 4 118 704
- US-A- 4 701 761
- IEEE TRANSACTIONS ON BROADCASTING. vol. 25, no. 4, December 1979, NEW YORK USpages 143 - 146; TAKIZAWA: 'REDUCTION OF GHOST SIGNAL BY USE OF MAGNETICABSORBING MATERIAL ON WALLS '

## Description

The present invention relates to a wave absorber constructed using a ferrite magnetic material, and, in particular, to a broad-band wave absorber in which ferrite members are arranged at a specific spacing on a conductive plate.

Much research has been performed on conventional wave absorbers that use ferrite, so much so that their capabilities are becoming well-known.

The construction of the wave absorber that has become a conventional standard is such that ferrite tiles (plates) are arranged on a conductive plate, as shown in Fig. 17.

US-A-4118704 discloses a variation in which some of the ferrite plates are removed in a regular pattern in an electric field direction to leave portions where the conductive plate is exposed (called vacant portions), as shown in Fig. 18.

In general, if such vacant portions are provided, characteristics the same as those of the structure of Fig. 17 can be obtained by making the thickness of the ferrite in the ferrite parts greater than that of the ferrite of Fig. 17, but the bandwidth characteristics cannot be expected to be improved thereby.

US-A-4701761 discloses a wave absorber which consists of a composite having alternate layers of metal and ferrite material, forming tiles which are separated at their edges from adjacent tiles by a narrow air gap. GB-A-776158 discloses an absorber for radio waves composed of lossy layers, the effective loss resistance of the lossy layers decreasing towards a base surface. GB-A-1170420 discloses an absorber arrangement comprising plural wall elements, each having an external surface with a conductive coating thereon, the surface resistance of which decreases in the direction of propagation of the incident energy.

To widen the bandwidth, some other technologies are required.

An embodiment of the present invention provides a wave absorber having a wider bandwidth.

The present invention was designed while taking the above points into consideration, with the aim of providing a broadband wave absorber that has a much broader bandwidth than a conventional absorber, that can be used in the VHF, UHF, and microwave bands, and that has excellent characteristics such that it can not only be used as an absorber with respect to waves polarized in the horizontal and vertical directions, it can also be used as a wave absorber for unidirectional-polarization use.

According to a first aspect of the present invention there is provided a wave absorber comprising plural rectangular plates of a ferrite magnetic material, the plates being mutually aligned at a spacing b on a radio-wave reflecting surface, the space between the plates exposing the radio-wave reflecting surface to incident radiation, the plates having a first dimension d extending outwardly from said surface, each of said plates having the same dimensions and a constant cross-section in the direction of the first dimension, a major dimension L extending on said surface and a minor dimension 2tₘ extending on said surface characterised in that the following relationships hold:${\text{L≧d≧2t}}_{\text{m}}$${\text{20t}}_{\text{m}} {\text{≧b>2t}}_{\text{m}}$

According to a second aspect of the present invention there is provided a broad band wave absorber of ferrite magnetic material, said absorber defining a plurality of rows of rectangular cavities of uniform section, said rows being disposed side-by-side whereby each cavity is separated from respective adjacent cavities by a wall thickness of 2tₘ, each cavity having an open mouth and a closed end, said end being closed by a respective portion of an electrically conductive surface, and each cavity further having a first dimension d perpendicular to said surface, the spacing between each wall of one cavity and the corresponding wall of respective adjacent cavities being b, wherein the following relationships hold:-${\text{20tm≧b>2t}}_{\text{m}}$${\text{d≧2t}}_{\text{m}}$

Thus there is disclosed a broad-band wave absorber wherein beams formed of a ferrite magnetic material are placed at an optimal spacing and are aligned in a lattice form in longitudinal and lateral directions on a conductive plate. A magnetic material of a specific thickness tₘ is formed into cylindrical blocks of a height d (where d ≧ tₘ) wherein an end surface thereof is polygonal, and the cylindrical blocks are provided with a radio-wave reflecting surface arranged in such a manner that this surface is perpendicular to the axial direction of the blocks, and the end surface of the blocks is approximately perpendicular to a direction from which radio waves are incident. The ferrite magnetic material could also be formed into rectangular prisms of thickness 2tₘ, height d, and length in the longitudinal direction thereof L, with the prisms aligned at a spacing b on a radio-wave reflecting surface, the direction of the height dimension of the prisms being approximately parallel to a radio-wave incidence direction, and the surfaces thereof of the dimensions 2tₘ and L being perpendicular to the radio-wave incidence direction, forming a plane parallel to a magnetic field direction of incident radio waves and the dimension L, wherein the following relationships hold:${\text{L ≧ d ≧ 2t}}_{\text{m}}$${\text{20t}}_{\text{m}} {\text{≧ b > 2t}}_{\text{m}}$

The reasons why it was considered that the present invention would broaden the bandwidth of the wave absorber are described below.

In the configuration of Fig. 1, since a surface with a small surface area is aligned perpendicular to the direction from which incident waves are incident, it can be expected that waves reflected from the interface with the ferrite will be reduced. This differs from the single-layer configuration shown in Fig. 17 in that, in the portions where there is ferrite, the ferrite portions and vacant portions are arranged alternately, then no plane waves can exit - transverse-magnetic (TM) waves are propagated. Therefore the interfaces with the ferrite ensures that the waves that are not propagated into free space, are converted into TM waves, increasing the absorption over a wide frequency range and thus broadening the bandwidth.

In other words, in the conventional wave absorber, a surface of the ferrite tiles with a large surface area is aligned perpendicular to the direction of incident radio waves. The wave absorber of the present invention, however, has the characteristic that the equivalent surface with the large surface area is aligned parallel to the direction of incident radio waves, and the resultant electromagnetic characteristics are dramatically different. To put it another way, if the dimensions of the magnetic tiles are defined as a length L, a height d, and a thickness t (where L > d > t), the conventional wave absorber has tiles aligned with L-d surfaces thereof perpendicular to the direction of incident radio waves, but the wave absorber of the present invention, on the other hand, achieves a much broader bandwidth by having tiles aligned with the L-t surfaces thereof perpendicular to the direction of incident radio waves.

As described above, by providing a construction consisting of blocks of a ferrite magnetic material shaped to specific dimensions and aligned at a specific spacing, the present invention can provide a broadband wave absorber able to absorb radio waves over a wide frequency range, by reducing wave reflection and by increasing absorption by TM wave.
Figs. 1(a), (b), and (c) are perspective views illustrating an embodiment of the present invention;
Figs. 2(a) and (b) are views of models used in a description of the embodiment of Fig. 1;
Fig. 3 is a graph of the absorption characteristics of the embodiment of Fig. 1;
Fig. 4 is a graph of the variation with height of the absorption characteristics of this embodiment of the present invention;
Fig. 5 is a graph of the variation with thickness of the absorption characteristics of this embodiment of the present invention;
Fig. 6 is a graph of a variation in the spacing of the absorption characteristics of this embodiment of the present invention;
Fig. 7 is a graph of absorption capability, showing the relationship between absorbent bodies and vacant portions used in the present invention;
Fig. 8 is a graph of absorption capability, showing the relationship between frequency and the K constants of the dispersion equation used in the present invention;
Fig. 9 is a graph of absorption characteristics when the product S of the kl and fl [MHz] of the dispersion equation is 8000 MHz;
Figs. 10(a), (b), and (c) are perspective and front views illustrating an embodiment configured of coaxial tubes, and a graph showing the characteristic thereof;
Figs. 11 to 13 are side and perspective views illustrating other embodiments of the present invention;
Fig. 14 is a perspective view of an embodiment of the present invention in which ferrite bars are inserted longitudinally and laterally;
Figs. 15 and 16 are perspective views of further embodiments of the present invention;
Fig. 17 is a perspective views of the configuration of a wave absorber that has become a conventional standard as known from US-A- 4 118 704; and
Fig. 18 is a perspective view of the configuration of an actual conventional wave absorber as known from US-A- 4 118 704.

The present invention will first be described with reference to the embodiment thereof shown in Figs. 1(a), (b), and (c); this embodiment will then be analyzed with reference to the model thereof shown in Figs. 2(a) and (b); the results of experiments will be described with reference to Figs. 3 to 9; and finally other embodiments of the present invention will be described with reference to Figs. 10 to 16.

The perspective view of Fig. 1(a) shows the essential details of an embodiment of the wave absorber of the present invention that uses horizontally and vertically polarized waves. Fig. 1(b) shows a wave absorber similar to that of Fig. 1(a), but in which the vertically aligned magnetic frames are removed and a conductive plate 1 that is in contact with the radio-wave reflecting surface is inserted into the thickness of each lateral frame, and Fig. 1(c) shows a further example in which the conductive plates 1 are omitted from within the ferrite frames.

The explanation that follows is based on the above structure for unidirectional-polarization waves.

The wave absorber of the present invention is configured of a stack of a large number of identical units of the same construction shown in Fig. 1. Each unit consists of ferrite plates 3 formed in a box shape on a conductive plate 2 that forms a radio-wave reflecting surface, the thickness of the ferrite plates 3 being 2tₘ, the spacing therebetween being b, and the height thereof being d; and the units are aligned on the conductive plate 2 in such a manner as to form a lattice. Since all of these units act in exactly the same manner, analysis thereof can be conducted by considering a single unit.

Fig. 2(a) shows a single-cell model used in such analysis. The symmetry of the overall structure means that it is possible to assume that a metal plate 1 can be inserted into the central portion of each ferrite plate, parallel thereto, without affecting in any way the magnetic field thereof. Therefore, the analysis below uses the model shown in Fig. 2(b).

In this analysis, the following equation is used to find »ᵣ, the relative permeability of each ferrite magnetic material:${\text{»}}_{\text{r}} {\text{= l + {K}}_{\text{l}} {\text{× f}}_{\text{l}} {\text{/ (f}}_{\text{l}} \text{+ jf)}}$
where f is frequency MHz and (l + kₗ) is the initial relative permeability under DC conditions.

In this equation, fl [MHz] corresponds to the frequency at which the imaginary part of the relative permeability becomes a maximum.

A value S, the product of kl and fl (i.e., kl × fl), is the quality of ferrite magnetic materials. Of the various compositions of ferrite is 10,000 MHz or less.

This analysis uses a value of 6000 MHz for the product S for ferrite. Therefore, if the value of kl is fixed, the value of fl [MHz] is automatically fixed.

This analysis is based on the use of ferrite whose value of kl is 1000 and fl is 6 MHz.

Since there is virtually no frequency dispersion in the permittivity εᵣ of ferrite, so this analysis is based on the assumption that there is no variation therein with the frequency, i.e., that:${\text{ε}}_{\text{r}} \text{= 16 - j0}$

It is known that, with a single-layer absorber using ferrite, the thickness that gives the best absorption is more-or-less constant, regardless of frequency, and that it is 8 mm if S is 6000 MHz.

In Fig. 3, curve A shows the absorption frequency characteristics for a single-layer absorber.

The wave absorber of the present invention has three parameters: the thickness 2tₘ of the ferrite plates, the spacing b between the ferrite plates, and the height d of the ferrite plates. Since it is not feasible to analyze all variations in these parameters, the description below relates to parameters at which the characteristics were best within the analyzed range: 2tₘ = 8 mm, b = 20 mm, and d = 20 mm. In Fig. 3, the absorption characteristic B for a wave absorber for which the above dimensions were selected is shown superimposed on the characteristic A of the conventional single-layer absorber.

In general, the reflectivity that is a characteristic of a wave absorber must be less than or equal to a permissible reflection coefficient. This analysis concerns evaluation at a frequency bandwidth that is 1% of the power level, i.e., at -20 dB or less.

It is clear from the characteristics curves of Fig. 3 that the wave absorber of the present invention has an extremely broad bandwidth.

It is also clear that if a wave absorber of this structure is formed with absorbent bodies of the same surface area as that of the single-layer absorber, roughly the same volume of ferrite as that of the single-layer absorber would be sufficient, proving that adoption of the structure of the present invention will result in a dramatic improvement in characteristics for the same quantity of ferrite.

As mentioned above, the absorber of the present invention has three parameters: the thickness 2tₘ of the ferrite plates, the spacing b between the ferrite plates, and the height d of the ferrite plates. Another parameter is (b - 2tₘ)/b, the proportion of the metal plate occupied by the empty portions between ferrite plates, hereinafter called the vacancy ratio.

Fig. 4 shows absorption frequency characteristics obtained by varying the height of the ferrite plates while keeping the thickness thereof constant at 8 mm and the spacing therebetween constant at 20 mm. It is clear from the curves of Fig. 4 that when the height d of the ferrite plates becomes less than 20 mm, the characteristic at higher frequencies becomes better, but, in contrast, the characteristic at lower frequencies worsens. Therefore, in this case, it is considered that the best characteristic occurs when the height d is 20 mm.

In a similar way, Fig. 5 shows absorption frequency characteristics obtained by varying the thickness of the ferrite plates, and Fig. 6 shows absorption frequency characteristics obtained by varying the spacing therebetween. In both cases, it was found that an optimal value existed, in roughly the same way as that described above for variations in thickness, and this optimal value was at b = 20 mm.

Fig. 7 shows absorption frequency characteristics obtained by keeping the thickness of the ferrite plates fixed at 20 mm, but varying both b and 2tₘ in such a manner that the vacancy ratio (b - 2tₘ)/b was constant at 60%.

The sample characteristics shown in the figure were obtained with b = 10 mm, 2tₘ = 4 mm; b = 20 mm,2tₘ = 8 mm; b = 30 mm, 2tₘ = 12 mm; and b = 40 mm, 2tₘ = 16 mm. It is clear that the best characteristic occurs when b = 20 mm and 2tₘ = 8 mm, showing that the vacancy ratio is not particularly meaningful as a parameter. In other words, with the vacancy ratio kept constant, variations in b and 2tₘ are far more important as effects on characteristics.

Now for a look at the absorption frequency characteristics obtained by varying the kl and fl [MHz].

Fig. 8 shows the characteristics obtained by using the above optimal structure at which the product S is fixed at 6000 MHz, but kl and fl [MHz] are varied.

As can be seen from the characteristics curves of Fig. 8, if the value of kl is increased while the product S is kept constant, the bandwidth broadens. In other words, the frequency at which the curve starts to fall below -20 dB is determined by Kₗ, whereas the frequency at which the curve starts to rise above -20 dB is determined by the configuration of the absorber.

Next is an investigation of the case in which the product S is varied.

Fig. 9 shows the absorption frequency characteristics obtained when the product S was 8000 MHz.

With S = 6000 MHz, the best characteristic was obtained when 2tₘ = 8 mm, b = 20 mm, and d = 20 mm, but with S = 8000 MHz, the best characteristic was obtained when 2tₘ = 6 mm, b = 15 mm, and d = 15 mm. Experiments with S = 8000 MHz produced the same result that the bandwidth was seen to broaden as kl increased.

In this way, although it is obvious that dimensions will vary with the permeability and frequency characteristics of the ferrite material used in the optimal structure according to the present invention, in most cases, if the product S of kl and fl is between 4000 MHz and 10,000 MHz, 2tₘ should be between approximately 3 mm and 12 mm, and b should be equal to d, with both being between approximately 12 mm and 30 mm.

Another embodiment of the present invention, based on exactly the same physical phenomenon as the above model but with a different structure consisting of coaxial conductive tubes, will now be described with reference to Fig. 10.

The wave absorber shown in Figs. 10(a) and (b) has an annular configuration of an inner diameter of 12 mm, a thickness of 1.5 mm, and a length of 5 mm. This absorber is aligned with a coaxial internal conductor 1 in front in the axial direction of a short-circuiting plate 2 of a circular, coaxial conductive tube 3. Measurements of the absorption frequency characteristics with respect to variations in length L of this wave absorber are shown in Fig. 10(c).

As can be seen from Fig. 10(c), the bandwidth within which the absorption is below the permissible reflection is much broader at a length of 20 mm, showing good match with analytic results.

Another alternative to the plate-shaped ferrite magnetic bodies of Fig. 1 is a circular or polygonal prismatic form, as shown in Fig. 11.

Furthermore, disposing pyramid type wave absorber as shown in Fig. 12 and that operates at frequencies above the upper limit of the wave absorber of the present invention, either to the front or between parallel flat of the present invention enables compounding to further broaden the band.

In addition, there was no large change in the characteristics even if there is the dielectric 4 shown in Fig. 13 disposed between the parallel flat plates 3 of the wave absorber of the present invention.

Fig. 14 is effective for horizontal and/or vertical polarized waves.

Fig. 15 shows another embodiment of the present invention, in which the shape of the end surfaces of the ferrite magnetic body is formed into a cylindrical shape so that it forms a perpendicular unit. This perpendicular unit uses ferrite having a thickness tₘ so that one side is a, and so that the other side is b. This perpendicular unit is formed as a cylindrical block with a height d.

Fig. 16 shows one portion of a wave absorber of a required area and in which the cylindrical blocks of Fig. 15 are overlapped in the direction of the one side a, and in the direction of the other side b.

The magnetic material used in the present invention can be ferrite of NiZn, MgZn or MnZn or the like, and moreover, can be materials, such as ferrite powder is mixed with glass, ceramic, rubber, plastic, carbon, paper, or fiber, etc.

## Claims

1. A wave absorber comprising plural rectangular plates (3) of a ferrite magnetic material, the plates being mutually aligned at a spacing b on a radio-wave reflecting surface (2), the space between the plates exposing the radio-wave reflecting surface to incident radiation, the plates having a first dimension d extending outwardly from said surface, each of said plates having the same dimensions and a constant cross-section in the direction of the first dimension, a major dimension L extending on said surface and a minor dimension 2tₘ extending on said surface characterised in that the following relationships hold:${\text{L≧d≧2t}}_{\text{m}}$${\text{20t}}_{\text{m}} {\text{≧b>2t}}_{\text{m}}$

2. A wave absorber according to claim 1, wherein said ferrite magnetic material is an NiZn-type ferrite with an initial permeability of at least 700, and said plates have said minor dimension 2tₘ≦8 mm and a said first dimension d≧20 mm.

3. A wave absorber according to claim 1, wherein said ferrite magnetic material is an MnZn-type ferrite with an initial permeability of at least 2000, and said plates have a said minor dimension 2tₘ≦8 mm and a said first dimension d≧35 mm.

4. A wave absorber according to any preceding claim, wherein a conductive plate (1) is disposed approximately in the center in the direction of the said minor dimensions of each of said plates (3) of said magnetic material, one edge of said conductive member (1) being exposed and the opposite edge thereof being connected to said radio-wave reflecting surface (2).

5. A wave absorber according to any one of claims 1-3 including a member (1) disposed within each of said plates (3) and projecting therefrom in a direction away from said reflecting surface (2), said member (1) being one of an electrically conductive material, a magnetic material, and an electrically resistive material.

6. A wave absorber according to any preceding claim wherein a dielectric (4) is disposed in the spacings between the plates (3).

7. A broad band wave absorber (3) of ferrite magnetic material, said absorber defining a plurality of rows of rectangular cavities of uniform section, said rows being disposed side-by-side whereby each cavity is separated from respective adjacent cavities by a wall thickness of 2tₘ, each cavity having an open mouth and a closed end, said end being closed by a respective portion of an electrically conductive surface (2), and each cavity further having a first dimension d perpendicular to said surface, the spacing between each wall of one cavity and the corresponding wall of respective adjacent cavities being b, wherein the following relationships hold:-${\text{20tm≧b>2t}}_{\text{m}}$${\text{d≧2t}}_{\text{m}}$

8. A wave absorber according to claim 7 wherein each cavity is defined by a respective member comprising said ferrite magnetic material, each said member having a wall thickness tₘ, and having a rectangular external periphery and a rectangular internal periphery.

## Patentansprüche

1. Wellenabsorbtionseinrichtung mit einer Vielzahl von rechteckförmigen Platten (3) aus Ferritmagnetmaterial, welche wechselseitig mit einem Abstand b auf einer radiowellenreflektierenden Fläche (2) ausgerichtet sind, wobei der Raum zwischen den Platten die radiowellenreflektierende Fläche einfallender Strahlung aussetzt, wobei die Platten eine erste Abmessung d haben, und zwar in Ausdehnung nach außen von der Fläche, wobei jede der Platten dieselben Abmessungen und einen konstanten Querschnitt in Richtung der ersten Abmessung hat, und zwar eine größere Abmessung L, welche sich auf der Fläche erstreckt und eine kleinere Abmessung 2tₘ, welche sich auf der Fläche erstreckt, dadurch gekennzeichnet, daß die folgenden Beziehungen gelten:${\text{L ≧ d ≧ 2t}}_{\text{m}}$${\text{20t}}_{\text{m}} {\text{≧ b > 2t}}_{\text{m}}$

2. Wellenabsorbtionseinrichtung gemäß Anspruch 1, wobei das Ferritmagnetmaterial ein Ferrit vom NiZn-Typ ist mit einer Anfangspermeabilität von zumindest 700, wobei die Platten die kleinere Abmessung 2tₘ ≦ 8 mm und die erste Abmessung d ≧ 20 mm haben.

3. Wellenabsorbtionseinrichtung gemäß Anspruch 1, wobei das Ferritmagnetmaterial ein Ferrit vom MnZn-Typ ist mit einer Anfangspermeabilität von zumindest 2000, wobei die Platten die kleinere Abmessung 2tₘ ≦ 8 mm und die erste Abmessung d ≧ 35 mm haben.

4. Wellenabsorbtionseinrichtung gemäß einem der vorstehenden Ansprüche, wobei eine leitende Platte (1) etwa in der Mitte der Richtung der kleineren Abmessungen von jeder der Platten (3) des Magnetmaterials angeordnet ist, wobei eine Kante des leitenden Elementes (1) der radiowellenreflektierenden Fläche (2) ausgesetzt und die entgegengesetzte Kante hiervon mit dieser verbunden ist.

5. Wellenabsorbtionseinrichtung gemäß einem der Ansprüche 1 bis 3, mit einem Element (1), welches innerhalb jeder der Platten (3) angeordnet ist und hiervon in einer Richtung weg von der reflektierenden Fläche (2) vorspringt, wobei das Element (1) aus einem elektrisch leitenden Material, einem magnetischen Material oder einem elektrischen Widerstandsmaterial besteht.

6. Wellenabsorbtionseinrichtung gemäß einem der vorhergehenden Ansprüche, wobei ein Dielektrikum (4) in den Räumen zwischen den Platten (3) angeordnet ist.

7. Breitband-Wellenabsorbtionseinrichtung (3) aus Ferritmagnetmaterial, wobei die Absorbtionseinrichtung eine Vielzahl von Reihen von rechteckförmigen Hohlräumen gleichförmigen Querschnittes definiert, wobei die Reihen Seite an Seite angeordnet sind, wodurch jeder Hohlraum von jeweiligen benachbarten Hohlräumen durch eine Wanddicke von 2tₘ getrennt ist, wobei jeder Hohlraum einen offenen Mund und ein geschlossenes Ende aufweist, wobei das Ende durch einen jeweiligen Abschnitt aus einer elektrisch leitenden Oberfläche (2) geschlossen ist, und wobei jeder Hohlraum weiterhin eine erste Abmessung d senkrecht zu der Oberfläche aufweist, wobei der Abstand zwischen jeder Wand von einem Hohlraum und der entsprechenden Wand der jeweiligen benachbarten Hohlräume b ist, wobei die folgenden Beziehungen gelten:${\text{20t}}_{\text{m}} {\text{≧ b > 2t}}_{\text{m}}$${\text{d ≧ 2t}}_{\text{m}}$

8. Wellenabsorbtionseinrichtung gemäß Anspruch 7, wobei jeder Hohlraum durch ein jeweiliges Element definiert ist, welches das Ferritmagnetmaterial aufweist, wobei jedes der Elemente eine Wanddicke tₘ hat und einen rechteckförmigen Außenumfang und einen rechteckförmigen Innenumfang aufweist.

## Revendications

1. Matière absorbante d'onde comprenant plusieurs plaques rectangulaires (3) d'une matière magnétique à base de ferrite, les plaques étant alignées mutuellement suivant un écartement b sur une surface réfléchissant les ondes radioélectriques (2), l'espace entre les plaques exposant la surface réfléchissant les ondes radioélectriques au rayonnement incident, les plaques ayant une première dimension d s'étendant vers l'extérieur à partir de ladite surface, chacune desdites plaques ayant les mêmes dimensions et une section transversale constante dans la direction de la première dimension, la plus grande dimension L s'étendant sur ladite surface et lape plus petite dimension 2tₘ s'étendant sur ladite surface, caractérisée en ce que les relations suivantes sont vérifiées :${\text{L ≧ d ≧ 2t}}_{\text{m}}$${\text{20t}}_{\text{m}} {\text{≧ b > 2t}}_{\text{m}} \text{.}$

2. Matière absorbante d'onde selon la revendication 1, dans laquelle ladite matière magnétique à base de ferrite est une ferrite de type NiZn, avec une perméabilité initiale d'au moins 700, et dans laquelle lesdites plaques ont comme plus petite dimension 2tₘ ≦ 8 mm et comme première dimension d ≧ 20 mm.

3. Matière absorbante d'onde selon la revendication 1, dans laquelle ladite matière magnétique à base de ferrite est une ferrite de type MnZn, avec une perméabilité initiale d'au moins 2.000, et dans laquelle lesdites plaques ont comme plus petite dimension 2tₘ ≦ 8 mm et comme première dimension d ≧ 35 mm.

4. Matière absorbante d'onde selon l'une quelconque des revendications précédentes, dans laquelle une plaque conductrice (1) est disposée approximativement au centre dans la direction desdites plus petites dimensions de chacune desdites plaques (3) de ladite matière magnétique, un bord de ladite plaque conductrice (1) étant apparent et son bord opposé étant relié à ladite surface réfléchissant les ondes radioélectriques (2).

5. Matière absorbante d'onde selon l'une quelconque des revendications 1 à 3, incluant un élément (1) disposé à l'intérieur de chacune desdites plaques (3) et dépassant de celles-ci en s'écartant de ladite surface réfléchissante (2), ledit élément (1) étant l'une d'une matière conductrice de l'électricité, d'une matière magnétique et d'une matière électriquement résistante.

6. Matière absorbante d'onde selon l'une quelconque des revendications précédentes, dans laquelle un diélectrique (4) est disposé dans les espaces entre les plaques (3).

7. Matière absorbante d'onde à large bande (3) faite d'une matière magnétique à base de ferrite, ladite matière absorbante définissant plusieurs rangées de cavités rectangulaires de section uniforme, lesdites rangées étant disposées côte à côte, ce par quoi chaque cavité est séparée des cavités adjacentes respectives par une épaisseur de paroi de 2tₘ, chaque cavité ayant une embouchure ouverte et une extrémité fermée, ladite extrémité étant fermée par une partie respective d'une surface conductrice de l'électricité (2), et chaque cavité comportant en outre une première dimension d perpendiculaire à ladite surface, l'écartement entre chaque paroi d'une cavité et la paroi correspondante des cavités adjacentes respectives étant b ; dans laquelle les relations suivantes sont vérifiées :${\text{20t}}_{\text{m}} {\text{≧ b > 2t}}_{\text{m}}$${\text{d ≧ 2t}}_{\text{m}} \text{.}$

8. Matière absorbante d'onde selon la revendication 7, dans laquelle chaque cavité est définie par un élément respectif comprenant ladite matière magnétique à base de ferrite, chacun desdits éléments ayant une épaisseur de paroi tₘ, et ayant une périphérie externe rectangulaire et une périphérie interne rectangulaire.
